

## UNITED STATES PATENT OFFICE.

KONRAD MÜLLER, OF LUNEBURG, GERMANY, ASSIGNOR TO THE FIRM B. ROOS & CO.  
OF BERLIN, GERMANY.

## METHOD OF MANUFACTURING MOLD POWDER.

No Drawing

Application filed November 21, 1924. Serial No. 751,413.

*To all whom it may concern:*

Be it known that I, KONRAD MÜLLER, a citizen of the German Republic, and residing at Luneburg, Germany, have invented 5 certain new and useful Improvements in a Method of Manufacturing Mold Powder, of which the following is a specification.

In former times witch-meal (lycopodium) has been employed as mold-powder, 10 but as its price is high various surrogates have been introduced by and by, as, for instance, carbonate of lime, kieselguhr, tripoli-powder, brown-coal, and a lot of other substances. As the chief property of the mold-powder must be its complete repulsion to 15 water, the substance used is soaked with a comparatively considerable amount of a suitable wax or oil, a suitable fatty acid, or the like, whereby it is rendered water-repulsive. 20 The quantity of the respective added substance (wax, etc.) amounts, as a rule, from 3 to 10%, but in some cases it is considerably greater.

Now, I have discovered that a large part 25 of the wax or other added water-repulsive substance can be saved if pieces of unglazed muffles or the like as used in connection with the burning of chinaware or clay-ware are ground, and this powder is used as a substitute for the carbonate of lime, kieselguhr, 30 etc., etc. Only about 1/2% of the wax, etc., is needed to render the composition completely water-repulsive and to impart it also the certain other properties necessary for a 35 useful mold-powder.

*Example.*—200 kg. of finely ground unglazed muffle-pieces or the like are mixed with 1 kg. of wax or a suitable equivalent, and with a small amount of a dyeing substance of such a color that the composition assumes a color like, or similar to, that produced by witch-meal, the mixing being effected preferably by means of a stirring-device and at a temperature of from 70 to 80°. 40 C. The mixing by stirring is continued for about 1 hour, when a homogeneous composition will be obtained that can be employed

as mold-powder either at once or after having been sifted.

I claim:

1. The method of producing a mold-powder, consisting in grinding unglazed fire clay muffle-pieces and mixing the powder obtained with wax at a temperature which is only a little higher than the fusing 55 temperature of the wax, substantially as set forth.

2. The method of producing a mold-powder, consisting in grinding finely unglazed fire clay muffle-pieces and mixing the powder obtained with about 1/2% of wax at a temperature which is only a little higher than the fusing temperature of the wax, substantially as set forth.

3. The method of producing a mold-powder, consisting in grinding unglazed fire clay muffle-pieces and mixing intimately the powder obtained with wax at a temperature which is only a little higher than the fusing temperature of the wax, substantially 65 as set forth.

4. The method of producing a parting powder consisting in grinding pieces of unglazed burnt fire clay and mixing the powder obtained with wax at a temperature 75 which is a little higher than the fusion temperature of the wax.

5. The method of producing a parting powder consisting in grinding pieces of unglazed burnt fire clay and mixing the powder obtained with about one-half per cent 80 of wax at a temperature which is a little higher than the fusion temperature of the wax.

6. As a new article of manufacture a parting powder consisting of a mixture of finely ground burnt unglazed fire clay with wax which has been incorporated at a temperature slightly above the fusion temperature 85 of the wax.

7. As a new article of manufacture a parting powder consisting of a mixture of finely ground unglazed muffle pieces with wax which has been incorporated at a tempera- 90

- ture slightly above the fusion temperature of the wax.
8. The method of producing a parting powder consisting in grinding pieces of unglazed burnt fire clay and intimately mixing the powder so obtained with a water repellent material.
9. The method of producing a parting powder consisting in grinding unglazed muffle pieces and mixing intimately the powder so obtained with a water repellent material.
10. As a new article of manufacture a parting powder consisting of finely ground burnt unglazed fire clay with which has been 15 thoroughly incorporated a water repellent material.

In testimony whereof I have affixed my signature.

KONRAD MÜLLER.